

Patented May 21, 1929.

1,714,035

# UNITED STATES PATENT OFFICE.

CARL MAULER, OF VIENNA, AUSTRIA.

## PROCESS FOR ASCERTAINING THE RESISTANCE TO RUSTING SHOWN BY IRON, STEEL, AND IRON ALLOYS.

No Drawing. Application filed July 11, 1927, Serial No. 205,057, and in Austria July 22, 1926.

This invention relates to a method or process for ascertaining systematically and quickly the degree of the absolute or relative resistance to rusting shown by iron, steel and 5 iron or steel alloys and its object consists in determining measurably the affinity of oxygen with respect to iron, steel and iron or steel alloys.

The known methods of testing steel and 10 its alloys are rather imperfect and fail to produce a reliable base of comparison. The microscopic and macroscopic methods do not yield more satisfactory results than those methods in which the loss of weight by corrosion, is made use of for determining the influence of oxygen upon iron or steel.

I have discovered, that to each alloy of iron and steel corresponds a certain characteristic and critical concentration and temperature of an appropriate chemical solution, at which the surface of the metal unites with the oxygen of the solution. I have further discovered, that this property affords a reliable means, never used heretofore, for 25 characterizing and measuring the absolute or the relative resistance to rusting in the case of the so-called rust-proof steels. The affinity of oxygen with respect to iron, iron and steel alloys is determined systematically 30 and gradually by my process. It indicates in a reliable manner the resistance against rusting, that is the relative or absolute rusting resistance.

The process according to the present invention consists in that I determine that temperature (which corresponds to the characteristic critical concentration of a hot oxygenous chemical solution at which the surface of the iron, steel or alloy specimens combines with the oxygen of the solution. For this object I preferably employ a watery solution, which contains an oxidizing agent and a certain amount of the reaction products, which are formed during the reaction between iron and the chemical solution and which hereinafter are termed reaction products the said solution being preferably in a boiling state.

The signs of oxidation on the specimens of 50 iron, steel or alloys appear in colours of different kind and in different shapes, viz as points or dots, lines or specks, distributed over the specimen to a greater or smaller extent. Sometimes the whole surface of the 55 specimen is covered therewith. This greatly

depends from the homogeneity of the alloys.

For determining the temperature I preferably use a thermometer and proceed in such a manner, that I immerse into the heated bath above mentioned all the specimens 60 which are to be examined. Now I further heat the bath preferably until it is boiling and remove from time to time the specimens from the bath after having noted the temperature of the latter. By examining 65 the specimens after their withdrawal from the bath I note at what temperature the oxidation has taken place. This temperature correspond to a certain critical concentration of the bath, because the same is open, so that 70 water continuously evaporates from the bath.

The observations may be made for instance from degree to degree. Usually the signs of oxidation appear suddenly as soon as the corresponding temperature and density in the 75 solution is attained. The colorations of the oxidized specimens are not in all cases the same but depend essentially on the chemical nature of the additions to the iron or steel.

As the baths which I employ mostly contain a caustic alkali, the same takes up carbonic acid from the air. In order to remedy this drawback I add caustic lime to the bath occasionally.

The invention may be carried out according to the following example:—

I prepare a hot solution of 100 parts of caustic soda solution of 33%, 10 parts of sodium nitrate and a small quantity of the reaction products and maintain the alkalinity 90 by adding caustic lime from time to time. The bath thus prepared is heated until it is boiling, and the specimens to be examined are placed simultaneously into the bath, thus under like or the same conditions, for instance by means of a dipping device. In order to obtain comparable results it is necessary, that the surfaces of the said specimens have been treated in like manner, for instance cleaned by means of emery. 100

Now I determine at what temperature and thus also at what concentration of the boiling solution the oxidation of the individual specimens begins, this being indicated by a coloration of the specimen.

For instance at the beginning of the process the boiling bath may have a temperature of 130 centigrade. I immerse the specimens into the bath and from time to time I note whether any of the specimens has oxidized. 110

I proceed in this way and as the bath gets more and more concentrated owing to boiling, the temperature will rise, so that finally for every specimen a temperature is reached at which oxidation commences. In this manner I obtain a schedule indicating at what temperature of the bath and thus also at what concentration of the bath the tested specimens begin to oxidize. I have found, that the conduct of the iron, steel and the iron or steel alloys in this bath constitutes a means for determining their resistance against rusting, so that the specimens which oxidize at the higher temperature in the bath

are also those specimens which in ordinary use do not rust so readily or quickly.

Therefore the process according to the present invention yield reliable indications for determining the resistance to the rusting of iron, steel and iron or steel alloys. It can be carried out within a short time and does not call for extensive and expensive arrangements.

*First example.*

25

Common iron and the rust-proof steels of well-known steel-works, treated in the bath above stated, showed the following figures:

|      |             |              |               |              |             |
|------|-------------|--------------|---------------|--------------|-------------|
| Iron | Steel No. I | Steel No. II | Steel No. III | Steel No. IV | Steel No. V |
|------|-------------|--------------|---------------|--------------|-------------|

show the first sign of oxidation at

|         |         |         |         |         |         |
|---------|---------|---------|---------|---------|---------|
| 144° C. | 160° C. | 173° C. | 189° C. | 205° C. | 216° C. |
|---------|---------|---------|---------|---------|---------|

*Second example.*

30

A steel alloy with the same contents of carbon and manganese, but containing different amounts of chrome as an alloy-addition gave the following test:

|        |    |    |    |     |     |
|--------|----|----|----|-----|-----|
| Chrome | 2% | 4% | 8% | 16% | 20% |
|--------|----|----|----|-----|-----|

showed the first sign of oxidation at

|         |         |         |         |                    |
|---------|---------|---------|---------|--------------------|
| 146° C. | 149° C. | 158° C. | 196° C. | None up to 210° C. |
|---------|---------|---------|---------|--------------------|

35

*Third example.*

If the chrome-steel alloy of 8% is systematically alloyed with nickel, vanadium, cobalt, titanium and so forth, I obtain a scale of different temperatures of oxidation, which immediately indicates whether the new alloy is more or less or not at all susceptible to oxidation.

Of course within the scope of the present invention may be employed also other oxidizing solutions, such as caustic potash solution added with an oxidizing agent. Instead of using sodium nitrate as an oxidizing means I may apply the nitrate of potassium or any other appropriate oxidizing substance.

50 I claim—

55 1. Process for ascertaining systematically and quickly the degree of absolute or relative rust-resistance of iron, steel and iron alloys, consisting in determining the affinity of oxygen to iron, steel and iron alloys by immersing the specimens to be examined into a hot oxidizing solution and measuring from time to time the temperature of the solution in order to determine the temperature at the moment at which the surface of the immersed specimen combines with the oxygen of the solution.

60 2. Process for ascertaining systematically and quickly the degree of absolute or relative rust-resistance of iron, steel and iron alloys,

70 consisting in determining the affinity of oxygen to iron, steel and iron alloys by immersing the specimens to be examined into a boiling alkaline solution, containing an oxidizing agent and a small amount of the reaction products produced by the action of the said solution on iron, and measuring from time to time the temperature of the solution in order to determine the temperature at the moment at which the surface of the immersed 75 specimen combines with the oxygen of the solution.

75 3. Process for ascertaining systematically and quickly the degree of absolute or relative rust-resistance of iron, steel and iron alloys, consisting in determining the affinity of oxygen to iron, steel and iron alloys by immersing the specimens to be examined into a hot solution composed of water, caustic soda, an oxidizing agent and reaction products produced by the action of the said solution on iron and measuring from time to time the temperature of the solution in order to determine the temperature at the moment at which the surface of the immersed specimen combines with the oxygen of the solution.

80 4. Process for ascertaining systematically and quickly the degree of absolute or relative dust-resistance of iron, steel and iron alloys, consisting in determining the affinity of oxy-

- gen to iron, steel and iron alloys by immersing the specimens to be examined into a hot solution composed of 100 parts of caustic soda solution of 33% calculated on caustic soda, 10 parts of sodium nitrate and a small amount of the reaction products produced by the action of the said solution on iron and measuring from time to time the temperature of the solution in order to determine the temperature at the moment at which the surface of the immersed specimen combines with the oxygen of the solution.
5. Process for ascertaining systematically and quickly the degree of absolute or relative rust-resistance of iron, steel and iron alloys, consisting in determining the affinity of oxygen to iron, steel and iron alloys by immersing the specimens to be examined into a boiling alkaline solution containing an oxidizing agent and a small amount of the reaction products produced by the action of the said solution on iron, regenerating from time to

time the alkalinity of the solution by adding an appropriate amount of caustic lime and measuring from time to time the temperature 25 of the solution in order to determine the temperature at the moment at which the surface of the immersed specimen combines with the oxygen of the solution.

6. Process for ascertaining systematically 30 and quickly the degree of absolute or relative dust-resistance of iron, steel and iron alloys, consisting in determining the affinity of oxygen to iron, steel and iron alloys by immersing the specimens to be examined into a 35 boiling alkaline solution, containing an oxidizing agent and measuring from time to time the temperature of the solution in order to determine the temperature at the moment at which the surface of the immersed specimen combines with the oxygen of the solution. 40

In testimony whereof I affix my signature.  
CARL MAULER.